

## UNITED STATES PATENT OFFICE

2,242,260

## LUBRICATING COMPOSITION

Carl F. Prutton, East Cleveland, Ohio, assignor,  
by mesne assignments, to The Lubri-Zol De-  
velopment Corporation, Cleveland, Ohio, a cor-  
poration of Delaware

No Drawing. Application January 22, 1937,  
Serial No. 121,827

7 Claims. (Cl. 252—48)

This invention relates, as indicated, to lubricants and more particularly to lubricating compositions capable of providing efficient lubrication under extreme pressure conditions, that is, of satisfactorily maintaining a lubricating film between bearing or other metallic surfaces operating under such extremely high pressures as would ordinarily cause seizing or scoring of such surfaces if a plain mineral lubricating oil, for example, were employed. These lubricating compositions are characterized by the fact that they are generally more effective and at the same time more stable than those used heretofore.

This application is a continuation in part of my copending application Serial No. 755,987, filed December 4, 1934 and co-pending application Serial No. 737,070, filed July 26, 1934.

This invention further relates to a method of preventing seizing or scoring of relatively moving bearing surfaces and of reducing the wear or friction between such surfaces. The addition of certain agents to lubricating compositions generally for the purpose of improving their extreme pressure characteristics is not new. It is generally recognized that the degree of effectiveness of extreme pressure addition agents is usually directly proportional to their chemical or physico-chemical action on the bearing surfaces in producing a film which usually has an anti-fluxing function in preventing actual metal to metal contact, and in addition, sometimes the function of producing a film which is more strongly attached to the metal surfaces than plain lubricating oils. Also, the action of the addition agents is to provide a film characterized by the fact that the coefficient of friction between the surfaces where such film is maintained is generally lower than when ordinary lubricants are employed.

While a certain amount of chemical or physico-chemical action by the addition agent upon the bearing surfaces is necessary and desirable in order that an extreme pressure film may be produced, the addition agent must, nevertheless, be sufficiently stable and relatively inactive so that its activity along this line remains dormant under ordinary conditions and is only activated under the conditions of extreme pressure where its effectiveness is required for the stated purpose. In certain types of use, such as in crank-cases of internal combustion engines, and in lubricants added to motor fuels and thus introduced into the apparatus to be lubricated through the combustion zone, such relatively high temperatures are encountered that the resultant conditions tend to either decompose or render undesirably active many types of addition agents which are accordingly not usable in such an environment.

It is also generally accepted that many plain

5 lubricating compositions such as refined mineral oil, due either to naturally occurring constituents in the base material or constituents in the finished product produced by refining processes, are relatively corrosive, particularly when used in conjunction with certain sensitive metals or alloys.

10 It is a principal object of this invention to provide a lubricating composition characterized by the fact that it contains an addition agent which may be effective not only for the purpose of imparting extreme pressure characteristics to the lubricant, but at the same time likewise effective as a corrosion inhibitor for certain active constituents which may either be originally present or added to the composition for certain specific results and which will otherwise be detrimentally active.

15 It is a further object of this invention to provide a lubricating composition which may be characterized by the fact that all of the above named desirable characteristics are imparted thereto by means of a single addition agent.

20 Other objects of this invention will appear as the description proceeds.

25 To the accomplishment of the foregoing and related ends, said invention, then, consists of the features hereinafter fully described, and particularly pointed out in the claims, the following description setting forth in detail certain embodiments of the invention, these being illustrative, however, of but a few of the various ways in which the principle of the invention may be employed.

30 35 Broadly stated, this invention comprises the use as and in lubricants of organic compositions containing phosphorus and sulphur. These compositions are generally of the type which may be produced by reacting organic compositions with phosphorus and sulphur-containing reagents.

40 45 More specifically, this invention contemplates the use for the above purposes of organic compositions which (before reacting with the above referred to reagents) may desirably contain an organic oxygen compound and preferably a compound including a hydroxyl group which may advantageously be attached to a benzenoid ring structure.

50 Throughout the ensuing description of this invention, the above described material indicated as usable either by itself as a lubricant or in minor amounts as an addition agent to other lubricating compositions for the purpose of improving the characteristics of the same will, for convenience, hereinafter be referred to as the addition agent.

55 As above indicated, the addition agent is of the type produced by reacting an organic composition with certain reagents which contain either separately in combined or elemental form, or in

combination, phosphorus and sulphur. The addition agent thus produced may, in most cases, be described as an organic composition containing both the elements, phosphorus and sulphur.

The type of organic base composition contemplated for use in the reaction above described, by which the addition agents are produced, is represented by the following examples:

I. Hydrocarbons, preferably containing more than four (4) carbon atoms 10

A. Chain type (acyclic)

(1) Paraffins, e. g.

Pentane

Hexane

Octane

Decane

Acyclic terpenes

(2) Olefines, e. g.

Hexylene

Di-butylene

Di-iso-butylene

Amylene

(3) Acetylenes, e. g.

Butine, crotonylene

Pentine, valerylene

Hexine, hexylene

Heptine, oenanthylidene

Octine, caprylidene

Decine, menthene

Dodecyldiene

B. Cyclic

(1) Cyclo-aliphatic, e. g.

(a) Naphthenes, e. g.

Cyclopentane

Cyclohexane

Cyclo-octane

(b) Cyclo-olefins, e. g.

Cyclobutene

Cyclopentene

Cyclohexene

(c) It will be noted that certain of the above, i. e., cyclohexane and cyclohexene, are also hydro-aromatic compounds, of which the following are additional examples:

The hydro-diphenyls  
The hydro-naphthalenes,  
e. g., hexa- and dodeca-  
hydro-naphthalenes tet-  
ra- and decahydronaph-  
thalenes

The hydro-anthracenes  
The hydro-phenanthrenes  
The hydro-retenes

(2) Aromatic, e. g.

Benzene

Di-phenyl

Naphthalene

Anthracene

Phenanthrene

Bridged ring hydrocarbons, e. g.  
aromatic terpenes such as  
pinene

Homologs of the above such as  
alkylated aromatic hydrocar-  
bons, e. g. methyl, ethyl, propyl  
and iso-propyl, butyl, ampl, etc.  
benzenes, diphenyls, naphtha-  
lenes, anthracenes, phenan-  
threnes—more specific exam-  
ples are toluene, xylene, ethyl-  
benzene, cumene, cymene  $\alpha$   
methyl naphthalene, retene

Aromatic hydrocarbons with one  
or more unsaturated side-  
chains, such as phenyl ethylene  
(styrene)

5 II. Naturally occurring, or commercially available  
complex compositions consisting principally  
of hydrocarbons

A. Petroleum and petroleum derivatives,  
such as crude mineral oils of paraffinic,  
naphthenic, or asphaltic character and  
from various sources including the  
Penn., Mid-Cont., and Coastal fields;  
and products refined from them, e. g.

Bright stock

Neutral or pale oils

Steam refined oils

Fuel oils

Kerosene

Gas oils

Gasolines

Paraffin wax (or petroleum wax)

Petrolatum

Solvent extracted fractions, e. g.

Edeleanu extract

Furfural extract

B. Hydrocarbon materials of non-mineral  
origin, e. g. hydrocarbon products of  
vegetable origin such as certain oils ob-  
tained from the distillation of wood,  
etc., e. g.

Retene oil

Turpentine

III. Oxygen-bearing organic compounds (includ-  
ing oxygen-bearing derivatives of hydro-  
carbons in Groups I and II above) may  
be classified according to the nature of at-  
tachment of the oxygen atom, viz:

(a) Directly attached to one or more  
carbon atoms, as in the case of:

(1) Ethers and analogous com-  
pounds,

(2) Compounds containing the



radicle, such as the alcohols  
and other derivatives of car-  
binol (including phenols, cre-  
sols, naphthols, etc.)

(3) Compounds containing the car-  
bonyl



radicle, such as amides, alde-  
hydes, ketones, organic acids,  
esters and salts of organic  
acids, thio-acids and esters of  
thio-acids.

(4) Compounds in which oxygen  
forms a part of the ring  
structure, e. g. furan and its  
derivatives, etc.,

(5) Compounds with an inorganic  
radicle where the oxygen is  
directly attached to a carbon  
atom

Arsenite

Hypochlorite

Phosphite

Thiophosphate

Thiophosphite

$\beta$ -Hydroxylamines

(b) Indirectly attached through the means of some other atom, i. e., in the form of an inorganic radicle, e. g.:

|                         | <i>Aliphatic</i> | <i>Aromatic</i>                               |
|-------------------------|------------------|-----------------------------------------------|
|                         | <i>Ethers</i>    |                                               |
| Arsenate                | 5                | Di-ethyl ethers                               |
| Chlorate                |                  | Propyl and isopropyl ethers                   |
| Chlorite                |                  | Butyl and isobutyl ethers                     |
| Cyanate                 |                  | Amyl ethers                                   |
| $\alpha$ -Hydroxylamine |                  |                                               |
| Nitrate                 | 10               |                                               |
| Nitrite                 |                  |                                               |
| Nitro                   |                  | Ethyl propyl ethers                           |
| Nitroso                 |                  | Methyl butyl ethers                           |
| Oxime                   |                  |                                               |
| Perchlorate             | 15               |                                               |
| Phosphate               |                  | Glycol ether (diethylene-glycol)              |
| Sulphate                |                  | Mono-alkyl esters of dihydric alcohols, e. g. |
| Sulphite                |                  |                                               |
| Sulphinic acid          |                  |                                               |
| Sulphone                | 20               |                                               |
| Sulphonic acid          |                  | Mono-methyl ester of ethylene glycol          |
| Sulphoxide              |                  |                                               |
| Thio-sulphate           |                  |                                               |

The following are specific examples of suitable oxygen-bearing compounds:

| <i>Aliphatic</i>                                | <i>Aromatic</i>      | <i>Ketones</i>                                                                                                                                    |
|-------------------------------------------------|----------------------|---------------------------------------------------------------------------------------------------------------------------------------------------|
| <i>Alcohols</i>                                 |                      | <i>Mixed ketones</i>                                                                                                                              |
| Methyl alcohol                                  | Benzyl alcohol       |                                                                                                                                                   |
| Ethyl alcohol                                   | Phenyl ethyl alcohol |                                                                                                                                                   |
| Propyl and iso-propyl alcohols                  |                      | Methyl-ethyl ketone                                                                                                                               |
| Butyl and iso-butyl alcohols                    |                      | Methyl propyl ketones                                                                                                                             |
| Amyl alcohols                                   |                      | Ethyl propyl ketones, etc.                                                                                                                        |
| Lauryl alcohol                                  |                      |                                                                                                                                                   |
| Cetyl alcohol                                   |                      |                                                                                                                                                   |
| Polyhydroxy alcohols; Dihydroxy alcohols, e. g. |                      |                                                                                                                                                   |
| Ethylene glycol                                 |                      | 40                                                                                                                                                |
| Di-ethylene glycol                              |                      |                                                                                                                                                   |
| Tri-hydroxy alcohols, e. g.                     |                      |                                                                                                                                                   |
| Glycerine                                       |                      |                                                                                                                                                   |
| <i>Phenols</i>                                  |                      | <i>Cyclo-ketones</i>                                                                                                                              |
| Monohydroxy, e. g. Phenol                       |                      | 45 Cyclohexanone                                                                                                                                  |
| Alkyl phenols, e. g. Cresols                    |                      |                                                                                                                                                   |
| Xylenols                                        |                      |                                                                                                                                                   |
| Ethyl phenols                                   |                      |                                                                                                                                                   |
| Propyl and iso-propyl phenol                    |                      | 50 Acetaldehyde                                                                                                                                   |
| Amyl phenols                                    |                      | Propyl aldehydes                                                                                                                                  |
| Phenyl phenols                                  |                      |                                                                                                                                                   |
| Naphthols                                       |                      |                                                                                                                                                   |
| Polyhydroxy, e. g. Dihydroxy, e. g.             |                      |                                                                                                                                                   |
| Dihydroxy benzenes                              |                      | 55 Fatty acids, e. g. Saturated:                                                                                                                  |
| Pyrocatechin (catechol)                         |                      | Acetic                                                                                                                                            |
| Resorcinol                                      |                      | Propionic                                                                                                                                         |
| Hydroquinone                                    |                      | Butyric                                                                                                                                           |
| Dihydroxy diphenyls                             |                      | Lauric                                                                                                                                            |
| Tri-hydroxy, e. g.                              |                      | Palmitic                                                                                                                                          |
| Tri-hydroxy benzenes                            |                      | Stearic                                                                                                                                           |
| Pyrogallol                                      |                      | Unsaturated:                                                                                                                                      |
| Hydroxy-hydroquinone                            |                      | Oleic                                                                                                                                             |
| Phloroglucinol                                  |                      | Hydroxy:                                                                                                                                          |
| Others, e. g.                                   |                      | Lactic                                                                                                                                            |
| Rufigallol                                      |                      | Ricinoleic                                                                                                                                        |
| <i>Acids</i>                                    |                      | <i>Aldehydes</i>                                                                                                                                  |
|                                                 |                      |                                                                                                                                                   |
|                                                 |                      | 50 Acetaldehyde                                                                                                                                   |
|                                                 |                      | Salicyaldehyde                                                                                                                                    |
|                                                 |                      | Naphthyl aldehydes                                                                                                                                |
| <i>Acids</i>                                    |                      | <i>Esters</i>                                                                                                                                     |
|                                                 |                      |                                                                                                                                                   |
|                                                 |                      | 70 Esters of an aliphatic alcohol (such as those listed above under "Alcohols") and a fatty acid (such as those listed above under "Acids") e. g. |
|                                                 |                      | Esters of a phenol (such as those listed above under "Phenols") and a fatty acid (such as those listed above under "Acids") e. g.                 |

| <i>Aliphatic</i> | <i>Esters</i> | <i>Aromatic</i>                      |                                                                                                                                                                                                                                                                                                                                                                                                                                                                      |
|------------------|---------------|--------------------------------------|----------------------------------------------------------------------------------------------------------------------------------------------------------------------------------------------------------------------------------------------------------------------------------------------------------------------------------------------------------------------------------------------------------------------------------------------------------------------|
| Methyl           |               | Phenyl, phenyl-phenyl, and naphthyl: | Hydrocarbon materials                                                                                                                                                                                                                                                                                                                                                                                                                                                |
| Ethyl            | Acetate       | Acetate                              | Petroleum derivatives, particularly mineral oil, for example                                                                                                                                                                                                                                                                                                                                                                                                         |
| Propyl           | Propionate    | Propionate                           | Bright stock (preferably Pennsylvania)                                                                                                                                                                                                                                                                                                                                                                                                                               |
| Butyl            | Butyrate      | Butyrate                             | Neutral or pale oils                                                                                                                                                                                                                                                                                                                                                                                                                                                 |
| Amyl             | Laurate       | Laurate                              | Oxygen-bearing organic compounds                                                                                                                                                                                                                                                                                                                                                                                                                                     |
| Lauryl           | Palmitate     | Palmitate                            | Phenol                                                                                                                                                                                                                                                                                                                                                                                                                                                               |
| Cetyl            | Stearate      | Stearate                             | Cresols                                                                                                                                                                                                                                                                                                                                                                                                                                                              |
| Ethylene         | Oleate        | Oleate                               | Diphenyl ether                                                                                                                                                                                                                                                                                                                                                                                                                                                       |
| Diethylene       |               |                                      | Stearic acid                                                                                                                                                                                                                                                                                                                                                                                                                                                         |
| Glyceryl         |               |                                      | Benzyl alcohol                                                                                                                                                                                                                                                                                                                                                                                                                                                       |
|                  |               |                                      | Lauryl alcohol                                                                                                                                                                                                                                                                                                                                                                                                                                                       |
|                  |               |                                      | Oxidized hydrocarbons including oxidized mineral oils                                                                                                                                                                                                                                                                                                                                                                                                                |
|                  |               |                                      | Naphthenic acid                                                                                                                                                                                                                                                                                                                                                                                                                                                      |
|                  |               |                                      | Methyl stearate                                                                                                                                                                                                                                                                                                                                                                                                                                                      |
|                  |               |                                      | Butyl stearate                                                                                                                                                                                                                                                                                                                                                                                                                                                       |
|                  |               |                                      | Methyl salicylate                                                                                                                                                                                                                                                                                                                                                                                                                                                    |
|                  |               |                                      | Oleic acid                                                                                                                                                                                                                                                                                                                                                                                                                                                           |
|                  |               |                                      | Fatty oils such as lard oil                                                                                                                                                                                                                                                                                                                                                                                                                                          |
|                  |               |                                      | Halogen-bearing organic compounds                                                                                                                                                                                                                                                                                                                                                                                                                                    |
|                  |               |                                      | Mono- and dichlor xylene                                                                                                                                                                                                                                                                                                                                                                                                                                             |
|                  |               |                                      | Mono- and dichlor cresol                                                                                                                                                                                                                                                                                                                                                                                                                                             |
|                  |               |                                      | Para- and orthochlorphenol                                                                                                                                                                                                                                                                                                                                                                                                                                           |
|                  |               |                                      | Monochlor pentane (chlor amyl phenol)                                                                                                                                                                                                                                                                                                                                                                                                                                |
|                  |               |                                      | Chlorinated diphenyl ether, for example trichlor diphenyl ether and hexachlor diphenyl ether                                                                                                                                                                                                                                                                                                                                                                         |
|                  |               |                                      | Mono- and dichlor benzyl alcohol                                                                                                                                                                                                                                                                                                                                                                                                                                     |
|                  |               |                                      | Methyl dichlor stearate                                                                                                                                                                                                                                                                                                                                                                                                                                              |
|                  |               |                                      | The reagents which may be employed with the above defined organic base compositions in producing the so-called addition agents, according to this invention, are, as previously indicated, characterized by their containing free or combined phosphorus and sulphur, either present in the same or different compounds and either in elemental or combined form. Those containing the above-named elements in combined form may generally be classified as follows: |
|                  |               |                                      | <i>Reagents</i>                                                                                                                                                                                                                                                                                                                                                                                                                                                      |
|                  |               |                                      | A. Phosphorus compounds                                                                                                                                                                                                                                                                                                                                                                                                                                              |
|                  |               |                                      | 1. Compounds of phosphorus and halogen                                                                                                                                                                                                                                                                                                                                                                                                                               |
|                  |               |                                      | Phosphorus chloride— $P_2Cl_4$                                                                                                                                                                                                                                                                                                                                                                                                                                       |
|                  |               |                                      | Phosphorus tri-chloride— $PCl_3$                                                                                                                                                                                                                                                                                                                                                                                                                                     |
|                  |               |                                      | Phosphorus pentachloride— $PCl_5$                                                                                                                                                                                                                                                                                                                                                                                                                                    |
|                  |               |                                      | Phosphorus dichlor trifluoride— $PCl_2F_3$                                                                                                                                                                                                                                                                                                                                                                                                                           |
|                  |               |                                      | 2. Compounds of phosphorus and oxygen                                                                                                                                                                                                                                                                                                                                                                                                                                |
|                  |               |                                      | Phosphorus trioxide— $P_2O_3$ (or $P_2O_5$ )                                                                                                                                                                                                                                                                                                                                                                                                                         |
|                  |               |                                      | Phosphorus tetraoxide— $P_2O_4$                                                                                                                                                                                                                                                                                                                                                                                                                                      |
|                  |               |                                      | Phosphorus pentoxide— $P_2O_5$ (or $P_4O_{10}$ )                                                                                                                                                                                                                                                                                                                                                                                                                     |
|                  |               |                                      | 3. Compounds of phosphorus, oxygen and halogen                                                                                                                                                                                                                                                                                                                                                                                                                       |
|                  |               |                                      | Phosphorus oxychloride $POCl_3$                                                                                                                                                                                                                                                                                                                                                                                                                                      |
|                  |               |                                      | Phosphorus trioxotetrachloride— $P_2O_2Cl_4$                                                                                                                                                                                                                                                                                                                                                                                                                         |
|                  |               |                                      | 4. Elemental phosphorus                                                                                                                                                                                                                                                                                                                                                                                                                                              |
|                  |               |                                      | B. Sulphur compounds                                                                                                                                                                                                                                                                                                                                                                                                                                                 |
|                  |               |                                      | 1. Sulphur and halogen                                                                                                                                                                                                                                                                                                                                                                                                                                               |
|                  |               |                                      | Sulphur monochloride— $S_2Cl_3$                                                                                                                                                                                                                                                                                                                                                                                                                                      |
|                  |               |                                      | Sulphur trichloride— $SCl_2$                                                                                                                                                                                                                                                                                                                                                                                                                                         |
|                  |               |                                      | 2. Sulphur and oxygen                                                                                                                                                                                                                                                                                                                                                                                                                                                |
|                  |               |                                      | Sulphur dioxide— $SO_2$                                                                                                                                                                                                                                                                                                                                                                                                                                              |
|                  |               |                                      | Sulphur trioxide— $SO_3$                                                                                                                                                                                                                                                                                                                                                                                                                                             |
|                  |               |                                      | Sulphur heptoxide— $S_2O_7$                                                                                                                                                                                                                                                                                                                                                                                                                                          |
|                  |               |                                      | 3. Sulphur, oxygen and halogen                                                                                                                                                                                                                                                                                                                                                                                                                                       |
|                  |               |                                      | Sulphur monoxotetrachloride— $S_2OCl_4$                                                                                                                                                                                                                                                                                                                                                                                                                              |
|                  |               |                                      | Sulphur pentoxydichloride— $S_2O_5Cl_2$                                                                                                                                                                                                                                                                                                                                                                                                                              |
|                  |               |                                      | Sulphuric oxychloride— $SO_2Cl_2$                                                                                                                                                                                                                                                                                                                                                                                                                                    |
|                  |               |                                      | Sulphurous oxychloride— $SOCl_2$                                                                                                                                                                                                                                                                                                                                                                                                                                     |

Esters of fatty acids derived from naturally occurring fatty oils and waxes, and of the hydrogenated acids derived from like sources, e. g.

Methyl, ethyl, butyl, etc. esters of coconut fatty acid, palm fatty acid, or the same after hydrogenation.

Naturally occurring, or commercially available complex oxygen-bearing organic compositions such as:

Non-mineral oils and waxes, e. g.

Fatty oils, including:

Animal oils,

Fish oils

Lard oil

Vegetable oils,

Cottonseed oil

Rape seed oil

Corn oil

Castor oil

Soya bean oil

Waxes of animal or vegetable origin:

Carnauba wax

Palm wax

Beeswax

Japan wax

Of the foregoing named organic base compositions, the following are among the more suitable:

|                                                                                                                                                                                                                                                                                                                        |    |                                                                                                                                                                                                                                                                                                                                                    |
|------------------------------------------------------------------------------------------------------------------------------------------------------------------------------------------------------------------------------------------------------------------------------------------------------------------------|----|----------------------------------------------------------------------------------------------------------------------------------------------------------------------------------------------------------------------------------------------------------------------------------------------------------------------------------------------------|
| 4. Elemental sulphur                                                                                                                                                                                                                                                                                                   |    | Fatty oils such as lard oil                                                                                                                                                                                                                                                                                                                        |
| <b>C. Phosphorus and sulphur compounds</b>                                                                                                                                                                                                                                                                             |    | Methyl salicylate                                                                                                                                                                                                                                                                                                                                  |
| 1. Compounds of phosphorus and sulphur alone                                                                                                                                                                                                                                                                           | 5  | Stearic acid                                                                                                                                                                                                                                                                                                                                       |
| Phosphorus disulfide— $P_2S_6$ (or $PS_2$ )                                                                                                                                                                                                                                                                            |    | Oleic acid                                                                                                                                                                                                                                                                                                                                         |
| Phosphorus trisulphide— $P_4S_3$ (or $P_2S_3$ )                                                                                                                                                                                                                                                                        |    | Diphenyl                                                                                                                                                                                                                                                                                                                                           |
| Phosphorus sesquisulphide— $P_4S_3$                                                                                                                                                                                                                                                                                    |    | Dichlor xylene                                                                                                                                                                                                                                                                                                                                     |
| Phosphorus pentasulphide— $P_2S_5$ (or $PS_10$ )                                                                                                                                                                                                                                                                       | 10 | Dichlor cresol                                                                                                                                                                                                                                                                                                                                     |
| Phosphorus heptasulphide— $P_4S_7$                                                                                                                                                                                                                                                                                     |    | Orthochlor phenol                                                                                                                                                                                                                                                                                                                                  |
| 2. Compounds of phosphorus, sulphur and halogen                                                                                                                                                                                                                                                                        |    | Monochlor amyl phenol                                                                                                                                                                                                                                                                                                                              |
| Phosphorus thiocloride— $PSCl_3$                                                                                                                                                                                                                                                                                       | 15 | Methyl dichlor stearate                                                                                                                                                                                                                                                                                                                            |
| Phosphorus thiobromide— $PSBr_3$                                                                                                                                                                                                                                                                                       |    | Chlordiphenyl                                                                                                                                                                                                                                                                                                                                      |
| Phosphorus thiobromide— $P_2S_3Br_4$                                                                                                                                                                                                                                                                                   |    |                                                                                                                                                                                                                                                                                                                                                    |
| 3. Compounds of phosphorus, sulphur and oxygen                                                                                                                                                                                                                                                                         |    |                                                                                                                                                                                                                                                                                                                                                    |
| Phosphorus sulphoxide— $P_4S_4O_6$                                                                                                                                                                                                                                                                                     |    |                                                                                                                                                                                                                                                                                                                                                    |
| 4. Compounds of phosphorus, sulphur and elements other than oxygen or halogen                                                                                                                                                                                                                                          |    |                                                                                                                                                                                                                                                                                                                                                    |
| Phosphorus thiocyanate— $P(CNS)_3$                                                                                                                                                                                                                                                                                     |    |                                                                                                                                                                                                                                                                                                                                                    |
| <b>D. Reagents containing elements equivalent to phosphorus and/or sulphur</b>                                                                                                                                                                                                                                         | 25 |                                                                                                                                                                                                                                                                                                                                                    |
| 1. Compounds of phosphorus and equivalents of sulphur, e. g. Se, for example                                                                                                                                                                                                                                           |    | <b>F. The product produced by reacting with phosphorus oxychloride (<math>POCl_3</math>)</b>                                                                                                                                                                                                                                                       |
| $P_2Se$                                                                                                                                                                                                                                                                                                                | 30 | (a) The reaction product of phenol with phosphorus pentasulphide ( $P_2S_5$ ) and                                                                                                                                                                                                                                                                  |
| $P_2Se_3$                                                                                                                                                                                                                                                                                                              |    | (b) The reaction product of orthochlorphenol with phosphorus pentasulphide.                                                                                                                                                                                                                                                                        |
| $P_2Se_5$                                                                                                                                                                                                                                                                                                              |    |                                                                                                                                                                                                                                                                                                                                                    |
| It will be noted that since the so-called addition agent produced by the above referred to reaction shall contain both phosphorus and sulphur, and advantageously phosphorus, sulphur and oxygen, organic compounds and the reagents selected shall be such as to produce the addition agent of the desired character. |    | The foregoing typical examples will be sufficient for those skilled in the art in utilizing the named reagents as well as their equivalents in producing the addition agents of this invention.                                                                                                                                                    |
| The following is a list of particularly suitable addition agents. Since the addition agents in the list are identified according to the organic compounds and reagents used in their preparation, it includes typical examples of suitable organic compounds and reagents.                                             | 35 | 35 The foregoing method of preparing the addition agent contemplated herein involves the use of reagents containing both phosphorus and sulphur or separate reagents which include both phosphorus and sulphur. Methods of preparing these addition agents other than that described above may be used, for example, by reaction of the following: |
| <b>A. Reaction products of the following organic compounds with phosphorus pentasulphide (<math>P_2S_5</math>):</b>                                                                                                                                                                                                    |    | A. Organic sulphur compounds with phosphorus-bearing reagents, e. g.                                                                                                                                                                                                                                                                               |
| Stearic acid                                                                                                                                                                                                                                                                                                           |    | (1) Mercaptans (including thio-alcohols and thio-phenols) with                                                                                                                                                                                                                                                                                     |
| Lauryl alcohol                                                                                                                                                                                                                                                                                                         | 50 | (a) $POCl_3$                                                                                                                                                                                                                                                                                                                                       |
| Benzyl alcohol                                                                                                                                                                                                                                                                                                         |    | (b) $PCl_3$                                                                                                                                                                                                                                                                                                                                        |
| Phenol                                                                                                                                                                                                                                                                                                                 |    | (c) $PSCl_3$                                                                                                                                                                                                                                                                                                                                       |
| Butyl stearate                                                                                                                                                                                                                                                                                                         |    | (d) $P_2O_5$                                                                                                                                                                                                                                                                                                                                       |
| Methyl salicylate                                                                                                                                                                                                                                                                                                      |    | (e) $PCl_5$                                                                                                                                                                                                                                                                                                                                        |
| Naphthenic acid                                                                                                                                                                                                                                                                                                        | 55 |                                                                                                                                                                                                                                                                                                                                                    |
| Diphenyl ether                                                                                                                                                                                                                                                                                                         |    | B. Organic phosphorus compounds with sulphur-bearing reagents, e. g.                                                                                                                                                                                                                                                                               |
| Cresylic acid (cresol)                                                                                                                                                                                                                                                                                                 |    | (1) Chlorinated organic phosphates or phosphites, (preferably with chlorine attached to aliphatic radicle) with                                                                                                                                                                                                                                    |
| Mineral oils such as bright stocks and neutrals (preferably Penn.)                                                                                                                                                                                                                                                     | 60 | Inorganic sulphide or polysulphide                                                                                                                                                                                                                                                                                                                 |
| Oxidized mineral oils                                                                                                                                                                                                                                                                                                  |    | (2) Organic phosphates and phosphites (preferably containing unsaturated organic radicles or products of incomplete reaction of organic hydroxy compounds with phosphorus-bearing reagents such as $POCl_3$ and $PCl_3$ ) with                                                                                                                     |
| Fatty oils such as lard oil                                                                                                                                                                                                                                                                                            |    | (a) $SCl_2$                                                                                                                                                                                                                                                                                                                                        |
| Chlorinated diphenyl ether, particularly trichlor diphenyl ether and hexachlor diphenyl ether                                                                                                                                                                                                                          | 65 | (b) $SCl_3$                                                                                                                                                                                                                                                                                                                                        |
| Mono- and dichlor benzyl alcohol                                                                                                                                                                                                                                                                                       |    | (c) Elemental sulphur                                                                                                                                                                                                                                                                                                                              |
| Para- and orthochlor phenol                                                                                                                                                                                                                                                                                            |    |                                                                                                                                                                                                                                                                                                                                                    |
| <b>B. Reaction products of the following organic compounds with phosphorus sulphochloride (<math>PSCl_3</math>)</b>                                                                                                                                                                                                    |    | Certain of the addition agents themselves, which have been previously generically defined as organic compounds containing both phosphorus and sulphur, may be generically, subgenerically and specifically classified in the following manner:                                                                                                     |
| Mineral oils such as bright stocks and neutrals (preferably Penn.)                                                                                                                                                                                                                                                     | 70 | (1) Organic compounds containing both phosphorus and sulphur                                                                                                                                                                                                                                                                                       |
| Oxidized mineral oils                                                                                                                                                                                                                                                                                                  |    |                                                                                                                                                                                                                                                                                                                                                    |
| Naphthenic acid                                                                                                                                                                                                                                                                                                        |    |                                                                                                                                                                                                                                                                                                                                                    |
| Methyl stearate                                                                                                                                                                                                                                                                                                        | 75 |                                                                                                                                                                                                                                                                                                                                                    |

- (2) Organic compounds containing phosphorus, sulphur and oxygen
- (3) Any of the foregoing compounds which contain a halogen.

A slightly different classification for certain types of the compounds usable as so-called addition agents, in accordance with this invention, is

- (1) Esters of phosphorus- and sulphur-containing acids, e. g.  
Esters of tri-thiophosphorus acid and  
Tetrathiophosphoric acid
- (2) Esters of phosphorus-, sulphur- and oxygen-containing acids, e. g.,  
Esters of thiophosphorus, thiophosphoric and  
Tri-thiophosphoric acids
- (3) Any of the previously mentioned compounds which contain a halogen.

Among the specific examples of addition agents contemplated for use in accordance with this invention which have been previously somewhat more generically defined, the following compounds may be mentioned, viz:

Tri-butyl thiophosphate  
Triphenyl thiophosphate  
Tri-benzyl thiophosphate  
Tri-cresyl thiophosphates, e. g., tri-(ortho-cresyl) thiophosphate  
Tri-butyl tri-thiophosphate  
Triphenyl trithiophosphate  
Tricresyl trithiophosphate  
Tributyl trithiophosphate  
Triphenyl trithiophosphate  
Tricresyl trithiophosphate  
Tri-(chlor ethyl) thiophosphate  
Tri-(ortho-chlor phenyl) thiophosphate  
Tri-(ortho-chlor phenyl) trithiophosphate  
Tri-(dichlor xylyl) thiophosphate  
Tri-(dichlor cresyl) thiophosphate  
Tri-(monochlor amyl phenyl) thiophosphate  
Tri-(chlorbenzyl) thiophosphate  
Tribenzyl trithiophosphate  
Tri-lauryl trithiophosphate  
Tri-(ortho-chlor phenyl) trithiophosphate

As previously indicated, the above named addition agents are usable either by themselves as lubricants or advantageously in small amounts as addition agents to other lubricating compositions. Their particular effectiveness in very small amounts for the purposes previously specified and hereafter explained in greater detail makes the so-called addition agents especially desirable for use in lubricating compositions comprising any of the well known oils usually used as lubricants, such as mineral oil, non-mineral oils such as animal and vegetable oils e. g. rape-seed oil, castor oil, or, for certain uses, desirable combinations of such oils.

It has been found that when a refined mineral lubricating oil base is used, the previously named desirable properties may be imparted thereto by the use of the named addition agents in amounts upwards of 0.10%. The amount of addition agent used in excess of the stated minimum depends of course upon the particular use for which the resultant composition is designed; in preparing a lubricant for use in the crank case of internal combustion engines, the composition will be found to give superior results if it contains from about 0.10% to about 2% of the addition agents.

If the resultant composition is to be used under

conditions of higher pressure where generally temperatures lower than those in a crank case are encountered, for example in lubricating heavily loaded gears and bearings, the addition agent may be present in greater amounts, i. e., up to 5 and, in certain cases, desirably up to 10 and 20% may be employed.

The principal advantages resulting from the use of the named addition agents in lubricating compositions of the character described are as follows: The addition agents will be found to impart substantial extreme pressure characteristics to the lubricant. The addition agents containing phosphorus, sulphur, halogen and oxygen will be found, in general, to be more effective than those containing only phosphorus, sulphur and oxygen, and the latter will generally be found to be more effective as extreme pressure addition agents than those which contain only phosphorus and sulphur.

Certain of the addition agents have an inherent property of inhibiting corrosion of metallic surfaces by such constituents as are usually present either by virtue of being contained in the mineral oil, created in the mineral oil during the refining process, or intentionally added thereto for the purpose of producing a particular result. The addition agents which contain halogen thus have the remarkable combination of desirable properties of imparting unusually high extreme pressure values to the composition, while at the same time rendering the same particularly stable and non-corrosive under ordinary conditions.

The oiliness factor of a lubricant, to which certain of the named addition agents have been added, has been found to be measurably improved over similar untreated lubricating compositions with which they have been compared.

The tendency of the lubricating composition to form sludges resulting either from oxidation or standing or under conditions of use is generally considerably reduced by the presence therein of the addition agent. If any sludge constituents are formed in the lubricating composition containing the addition agents, the latter have a marked tendency to render harmless such constituents so that even so formed, their presence in the composition is not objectionable.

Certain of the named constituents have been found to very materially improve the viscosity index and cold test characteristics of mineral lubricating oils to which they have been added.

The stability and volatility of the addition agents should be such that under conditions encountered in service the concentration of the addition agent in the lubricant will not be substantially reduced because of its loss by evaporation or by decomposition.

For most uses the addition agent should have a vapor pressure less than atmospheric at a temperature of 140° C.; and if the lubricant is to be subjected to elevated temperatures in use, less than atmospheric at 170° C.

The stability of the addition agent should be such that decomposition shall be negligible at temperatures to which the lubricant will be exposed in service.

By the term "non-corrosive" as used herein and in the appended claims is meant such forms of the addition agents as will not react chemically to a substantial and continuing extent with the bearings and other metallic parts exposed to the lubricant excepting under conditions of extreme pressure and the like, nor cause damaging corrosion of such metallic parts.

The foregoing statements as to non-corrosiveness, stability and volatility of the addition agents applies particularly to compositions made in accordance with this invention and used as lubricants and especially when such lubricants are employed under conditions of extreme stress such as imposed by high temperature, extremely high pressure and the like. There are, however, certain uses such as in metal working, die drawing and the like where relatively more active, i. e., relatively corrosive, addition agents of the character referred to herein may be employed to advantage.

While the lubricating compositions which have been described herein as illustrating one embodiment of the invention have been generally referred to as "oils," i. e., liquids, this invention is, however, also applicable to the solid and semi-solid types of lubricants commonly referred to in the trade as greases, bodied oils, etc. In this connection, it should be noted that certain of the addition agents contemplated for use herein for the purpose of imparting extreme pressure characteristics to the lubricant may be employed for the additional purpose of bodying or thickening the lubricant to which they are added.

Other modes of applying the principle of my invention may be employed instead of the one

explained, change being made as regards the materials employed in carrying out the process, provided the ingredient or ingredients stated in any of the following claims or the equivalent of such stated ingredient or ingredients be employed.

5 I, therefore, particularly point out and distinctly claim as my invention:

1. A lubricating composition comprising a halogenated aromatic thiophosphate.

10 2. A lubricating composition comprising a major proportion of mineral oil and a minor amount of a halogenated aromatic thiophosphate.

15 3. A lubricating composition comprising a major proportion of mineral oil and a minor proportion of tri(orthochlorphenyl) thiophosphate.

4. A lubricating composition comprising a major proportion of mineral oil and a minor amount of tri(monochlor amyl phenyl) thiophosphate.

20 5. A lubricating composition comprising a major proportion of mineral oil and a minor amount of a chlor-phenyl thiophosphate.

6. A lubricating composition comprising a major proportion of mineral oil and a minor amount of a chlor-benzyl thiophosphate.

25 7. A lubricating composition comprising a major proportion of mineral oil and a minor amount of tri(chlor-benzyl) thiophosphate.

CARL F. PRUTTON.